

Patented Aug. 24, 1926.

1,596,999

# UNITED STATES PATENT OFFICE.

BY RAMJI D. SAKLATWALLA, OF CRAFTON, PENNSYLVANIA.

## PRODUCTION OF LOW-CARBON IRON-CHROMIUM ALLOYS.

No Drawing.

Application filed March 11, 1922. Serial No. 543,083.

The present invention relates to the production of low-carbon iron-chromium alloys and has for its object the production of low-carbon iron-chromium alloys directly 5 from the chrome ore and at lower temperatures than those heretofore employed. The invention is particularly applicable to the production of low-carbon ferro-chromium and will be described with particular reference to it, it being understood however that the invention is applicable to other low-carbon iron-chromium alloys, such for example as chrome steels or irons.

In the manufacture of ferro-chromium, 15 the most commonly used ore is chromite, in which the chromium occurs as the sesquioxide  $\text{Cr}_2\text{O}_3$  in combination with iron in the form of ferrous oxide  $\text{FeO}$ . As invariable constituents of chromite, besides the  $\text{Cr}_2\text{O}_3$  and  $\text{FeO}$  contents, there are always present certain percentages of alumina ( $\text{Al}_2\text{O}_3$ ) and magnesia ( $\text{MgO}$ ) which render the chromium content very refractory to ordinary processes of reduction.

25 The reduction of the chromium content by means of carbon and separation of metal from the gangue can be effected at comparatively high temperature, when the oxygen, originally combined with the chromium, is removed only to be more or less replaced by the element carbon. The result of such a reduction is, therefore, a low grade product, containing approximately eight to four percent carbon, depending upon the amount of 35 carbon used, in theoretically calculated proportion or less, the yield naturally being lower with the lower carbon percentage.

The reduction of chromite by means of metallic reducing agents, such, for example, 40 as silicon, is carried out, at the present time, only in an electric furnace, at high temperature, under expenditure of considerable electrical energy; as, in spite of the exothermicity of the reduction reaction, considerable extraneous heat is required to be 45 added, to enable the refractory constituents alumina and magnesia, present in the ore, to form into a liquid slag, allowing through separation of the metal in regulin form. A 50 further disadvantage of this necessity of using an electric furnace for the carrying out of the process is the opportunity afforded to the reducing mixture of coming in contact with and picking up carbon from 55 the electrodes, thus lowering the quality of the metal produced. For this reason, it has

been, up to now, necessary, for the production of low-carbon ferro-chromium, to resort to the expediency of refining a higher carbon content alloy. This refining is accomplished by oxidizing the carbon content by gaseous, solid, or molten oxidizing agents. During such a process, however, a certain percentage of the chromium is oxidized simultaneously with the carbon and is lost, 60 rendering the operation very uneconomical.

In accordance with my method, the above deficiencies are obviated, and the chromite is reduced to low-carbon ferro-chromium with a complete regulin separation of the 70 metal by means of temperatures which are attainable in the ordinary combustion-heated furnace, such as a gas or coke-fired reverberatory or crucible furnace. If a combustion-heated furnace is used, the 75 higher cost of electric furnace operation may be eliminated, as well as the disadvantage of the absorption of carbon into the metal from the electric furnace electrodes. If an electric furnace is used, the process 80 may be carried out at a lower temperature than that hitherto employed, with consequent economy in furnace operation and less tendency to absorb carbon from the electrodes. The separation of the metal in 85 regulin form and the formation of a fluid slag without the aid of the high temperatures hitherto employed is made possible by the addition to the reduction mixture of a flux which will combine with the refractory constituents of the chromite and form 90 a slag which is fluid at the lower reduction temperatures, such as are attainable in a combustion-heated furnace. The flux preferably contains a material, such as a fluoride, 95 which will produce a slag which is liquid at the desired temperature. The added fluxing materials combine exothermically with the silica produced by the oxidation of the silicon and with the refractory constituents 100 of the ore, and thus augment the temperature produced by the reduction reaction. Furthermore, the compounds caused by the combining with the fluxing material and the silica and refractory constituents of the ore 105 have a low melting point and a low specific heat.

The fluxing material having the above indicated desirable qualities may be formed of a mixture of about equal amounts of lime 110 and fluorspar. The mixture of lime and fluorspar is added to the reduction mixture

which consists of chromite with silicon in theoretical proportions necessary for the reduction of its  $\text{Cr}_2\text{O}_3$  and  $\text{FeO}$  contents. The amount of lime ( $\text{CaO}$ ) to produce the desired result has been found to be between 50% and 70% by weight of the silicon (Si) employed for reduction, depending on the amount of the other bases present in the chromite. The quantity of fluorspar most 10 beneficial to the reaction has been found to be, in amount, about equal to that of the lime or in a slight excess of the lime. Other metallic oxides, such as ferric-oxide and manganese dioxide, may be used and produced by exothermic reactions similar low melting compounds in the presence of fluorspar. Such other metallic oxides may 15 replace in molecular proportions a part of the lime in the lime fluorspar mix. The 20 addition of boron trioxide up to about 5% of the lime accelerates the reaction, the generation of exothermic internal heat and the separation of the metal from the slag.

The term "silicon" as used herein, is intended to include not only a substantially 25 pure silicon, but also silicon-bearing alloys, such, for example, as ferro-silicon. It has also been found that parts of the silicon may be replaced by equivalent proportions of 30 other metallic reducing agents, such as manganese, aluminum, magnesium, calcium, etc.

While the preferred embodiment of the process has been specifically described, it is 35 to be understood that the process is not limited to its preferred embodiment, but may be embodied in other processes, within the scope of the following claims.

I claim:

40 1. The process of making iron-chromium alloys, which consists in smelting at a temperature attainable in a combustion heated furnace chrome ore and silicon together with lime and fluorspar in sufficient amounts 45 to render the slag liquid at temperatures at-

tainable in a combustion heated furnace, substantially as described.

2. The process of making iron-chromium alloys, which consists in smelting at a temperature attainable in a combustion heated 50 furnace chrome ore and silicon together with lime, fluorspar and boron trioxide in sufficient amounts to render the slag liquid at temperatures attainable in a combustion heated furnace, substantially as described. 55

3. The process of making iron-chromium alloys, which consists in smelting at a temperature attainable in a combustion heated furnace chrome ore and silicon together with a flux-forming mixture containing about 60 50%-70% by weight of lime of the silicon present and an approximately equal amount of fluorspar, substantially as described.

4. The process of making iron-chromium alloys, which consists in smelting at a temperature attainable in a combustion heated furnace chrome ore and silicon together with lime and a fluoride in sufficient amounts to render the slag liquid at temperatures attainable in a combustion heated furnace, 70 substantially as described. 65

5. The process of making iron-chromium alloys, which consists in smelting in a combustion heated furnace chrome ore and silicon together with lime and a fluoride in 75 sufficient amounts to render the slag liquid at temperatures attainable in a combustion heated furnace, substantially as described.

6. The process of making iron-chromium alloys, which consists in smelting at a temperature attainable in a combustion heated furnace chrome ore and silicon together with lime and fluorspar in sufficient amounts to render the slag liquid at temperatures attainable in a combustion heated furnace, 80 substantially as described. 85

In testimony whereof I have hereunto set my hand.

BYRAMJI D. SAKLATWALLA.